

# United States Patent Office

2,900,340

Patented Aug. 18, 1959

1

2,900,340

## ANHYDROUS CALCIUM BASE GREASES CONTAINING FREE FATTY ACID

Thomas W. Martinek and Ernest T. Fronczak, Crystal Lake, Ill., assignors to The Pure Oil Company, Chicago, Ill., a corporation of Ohio

No Drawing. Application December 31, 1954  
Serial No. 479,244

13 Claims. (Cl. 252—40)

This invention relates to anhydrous calcium soap grease and to the method of preparing the same.

Calcium soap greases made in the conventional manner from fatty acids or glycerides such as oleic and stearic acids or glycerides and mixtures thereof, require the presence of water in order to make the grease homogeneous. In the absence of water, the soap precipitates from the oil. However, the presence of water in the grease is objectionable because such greases have a low dropping point and as a result the use of such greases is limited to operating temperatures below 150° F. One method of overcoming this drawback is to replace the water by an association agent such as calcium acetate. Another method is set forth in Patent No. 2,607,734, wherein there is disclosed a method for making anhydrous calcium grease in which an hydroxy fatty acid is used in the preparation of the soap stock. Although greases made in accordance with this patent exhibit satisfactory dropping point and yield characteristics, they have the disadvantage of being rather expensive and produce a grainy structure unless subjected to a vigorous milling operation. The grease product of Patent No. 2,607,735 is similar to that of Patent No. 2,607,734, except that the former additionally contains a calcium salt of a low molecular weight acid. The grease of Patent No. 2,607,735 is subject to the same deficiencies as that of Patent No. 2,607,734.

We have now discovered that anhydrous calcium soap greases having high dropping points and high yields, and which are smooth and of a homogeneous structure with good stability without milling, can be prepared by using a mixture of high molecular weight hydroxy fatty acids such as hydroxy stearic acid, and conventional high molecular weight non-hydroxy fatty acids having not more than one unsaturated linkage in the molecule, such as oleic, behenic, erucic, and arachidic acids, in the preparation of the soap stock. Uniform results in the preparation of the grease are assured by controlling the free acidity so that the ratio of soap to free fatty acid in the mixture during grease processing is about 20 parts by weight of soap to from 0.3 to 1.85% parts of free fatty acid. Not only are such greases of uniform quality but they are substantially equal to straight hydroxy stearic acid greases in dropping point and other desirable characteristics and yet more economical to prepare because of the lower cost of the fat or fatty acid and the lower cost of processing due to the fact that processing time is considerably reduced and extensive milling is not necessary. In some cases the yield is higher. Moreover, the grease exhibits improved compatibility with all types of mineral oils over that exhibited by similar grease not having requisite free fatty acids present during preparation.

One object of this invention is to prepare a multi-purpose, stable anhydrous calcium soap grease.

Another object of this invention is to prepare calcium soap grease of high dropping point and yield.

Still another object of this invention is to prepare an-

2

hydrous calcium soap grease of controlled free acidity and desirable dropping point, yield characteristics and compatibility with mineral oils at a lower cost than heretofore.

Yet another object of this invention is to prepare uniformly desirable anhydrous calcium soap grease of controlled free acidity at a low cost by regulating the free acid content during preparation.

A particular point of novelty of this invention is the 10 step of controlling the free fatty acid concentration of said grease during its preparation in order to completely assure production of a superior anhydrous calcium soap grease. It has been found that when said acidity is not kept within rigid bounds during processing, said processing may be difficult and phase separation may occur, so that an unsatisfactory inferior grease product may result. A critical range of free fatty acids must be present at all times after the introduction of the soap constituents to the base oil in order to assure production of the desired grease.

In preparing grease in accordance with our invention, we may employ equally advantageously as the base oil any solvent-refined or conventionally-refined hydrocarbon oil or lubricating oil derived from petroleum oils produced from a Pennsylvania, Mid-Continent, Coastal or other source. The composition of the base oil may vary. The oil may be prepared from a single fraction or admixture of several fractions of lubricating oil and/or extracts thereof. Thus, solvent-refined neutral and bright stocks oils, that is, neutral and bright stock refined with phenol, furfural, nitrobenzene or similar solvents, may be used, as may the extracts obtained from such solvent refining processes. The grease of this invention is thus contrasted with a grease of similar 35 composition but not containing the above-described required concentration of free fatty acids, in that said latter grease is usually obtained in higher yield for a given amount of soap when extract of high aromatic content from the solvent refining of mineral oil bright stock with phenol, furfural, nitrobenzene or similar solvent is present in the base oil. The grease of this invention is prepared with equal facility no matter what base oil or base oils are used. In addition, after preparation of the grease of this invention, thinning of said grease may be accomplished with any one or mixture of two or more of the above-mentioned types of oils without fear of incompatibility of said grease with the oil or oils.

We prefer to prepare a slurry of lime and fatty acids in the base oil. If the base oil has residual acidity due to naphthenic and possibly other acids present, said residual acidity is first just neutralized with aqueous sodium hydroxide at about 170° F. to 190° F. in order that the lime, which is later added will not react with these acids.

After the base oil is neutralized with aqueous sodium hydroxide solution, sufficient fatty acids are added thereto in order to give a finished grease base having approximately 20 percent by weight of lime soap therein. The fatty acids are added to the heated and neutralized base oil at a temperature of about 170–190° F., followed immediately by the addition of a slurry of hydrated lime in oil. The oil used for the slurry is preferably a neutral oil fraction. The amount of lime should be sufficient to theoretically neutralize all but 0.3–1.85% by weight of total composition of all fatty acids present in the mixture. Alternatively, the fatty acids may be theoretically completely neutralized and additional fatty acids may be added later on in the process. After the addition of the lime slurry, the temperature of the mixture rises due to the exothermic reaction between the lime and the fatty acids. The rise in temperature of the mixture is controlled so that the mixture is kept at approximately

210-212° F. until foaming subsides and the reaction is completed. This usually takes place in less than one hour. The mixture is then by the ASTM titration method for acid number employing phenolphthalein as the indicator, or by any other suitable means of determining acidity.

After a determination of the acidity of the mixture, an adjustment in the acidity is made by the addition of the requisite amount of fatty acids to bring the free fatty acid concentration up to 0.3-1.85% by weight, calculated on the basis of the grease containing approximately 20% by weight of soap. Thus, if the calcium soaps present in the grease mixture at the time of testing represent 40% by weight of the mixture, then 0.6-3.7% by weight free fatty acids should be present. If, conversely, the percent by weight of soaps present is 10% then 0.15-0.9% by weight of the free fatty acids are necessary. Thus, the weight ratio of calcium soap gelation agent in the mixture to free fatty acids during preparation of the grease is 20:0.3-1.85. After the free fatty acid is properly regulated, the temperature of the grease mixture is then slowly increased to approximately 230° to 275° F. and the mixture is cooked at this temperature until the grease is substantially dehydrated and a smooth, clear plastic grease is obtained. The addition of the fatty acids keeps the grease from separating into two phases during the dehydration process. The cooking stage will usually require a considerably shorter period of time than six hours. The grease base may then be diluted with further quantities of the mineral base oil or oils to desired consistency and a finished grease is obtained which does not require milling.

#### Example I

As an example of grease prepared in accordance with our invention, a grease of the following formulation was prepared:

| Raw Materials                                   | Wt. Percent | Grams  |
|-------------------------------------------------|-------------|--------|
| Hydrogenated Castor Oil Acids <sup>1</sup>      | 1.985       | 114.8  |
| Arctic Red Oil <sup>2</sup>                     | 1.985       | 114.8  |
| Hydrated Lime                                   | 0.553       | 30.6   |
| Water                                           | 0.081       | 4.5    |
| Caustic Soda                                    | 0.027       | 1.5    |
| Solvent Refined Bright Stock <sup>3</sup>       | 77.248      | 4272.0 |
| Solvent Refined Neutral (200 Vis.) <sup>4</sup> | 18.119      | 1002.0 |

<sup>1</sup> Hydrogenated castor oil acids comprises mainly hydrogenated ricinoleic acid, the principal constituent of castor oil. Said hydrogenated ricinoleic acid is 12-hydroxy-stearic acid. Also, high molecular weight saturated acids are present in small amount, such as stearic acid.

<sup>2</sup> Arctic red oil is mainly oleic acid and may contain minute quantities of saturated higher molecular weight fatty acids.

<sup>3</sup> Solvent refined bright stock is bright stock which has been subjected to solvent extraction with phenol.

<sup>4</sup> Solvent refined neutral oil (200 vis.) has been subjected to solvent refining with phenol.

As can be seen from the above formulation, the total content of calcium soaps was approximately 4%. The grease was prepared by the following procedure:

Bright stock in the amount of 300 grams was charged to a grease kettle. Heat was applied and agitation started. When the bright stock reached a temperature of 170° F., a solution of all the caustic soda in all the water was added to the kettle. The fatty acids, that is, 109.8 grams of the hydrogenated castor oil acids and 109.8 grams of the arctic red oil, were then added while the kettle mixture was held at 190° F. After agitation, and while the resulting mixture was still held at 190° F. a lime slurry comprising 30.6 grams of the hydrated lime in 100 grams of the neutral oil was then added with stirring. This was followed by the addition of 80 grams of wash neutral oil, that is, oil utilized to wash the container which formerly contained the lime slurry.

Upon addition of the slurry, the temperature of the reaction mix climbed to about 202° F., due to the exothermic reaction between the hydrated lime and the fatty acids. Heat was applied to raise the batch temperature to 212° F. and said temperature was then maintained for

approximately 15 minutes. Additional heat was then applied to the batch to dehydrate the grease. When the batch temperature reached 214° F., the grease started to separate into two phases. On determination of the acidity of a sample of said grease at this point it was found to be 1.79% w. as oleic. An additional 5 gram amount of each acid was then added, that is, a total of 114.8 grams of hydrogenated castor oil acids and arctic red oil. The acidity was thus adjusted to a weight ratio of calcium soaps to free fatty acids of approximately 20:1.85.

The increased free fatty acids immediately caused the grease to assume its former homogeneous appearance and dehydration progressed smoothly as the temperature of the batch was increased. The grease gradually became clearer and tougher until at 240° F., 1.5 hours after the addition of lime slurry, a translucent, light green, very tough and smooth plastic grease was obtained. This grease was then diluted with the balance of the mineral oils to a final soap concentration of 4.0% by weight and a final free fatty acid concentration of about 0.39% by weight. Total time for processing was six hours.

The final grease had an ASTM tapered-hole disc penetration of 153 unworked, 155 worked and 152 at 2000 strokes.

The grease was found to be particularly suitable as a track-roller grease for continuous track vehicles and resembled in physical appearance aluminum-soap greases, but was more stable to working and less sensitive to changes in temperature than said aluminum-soap greases.

#### Example II

A further non-limiting example of the grease of our invention is a grease of the following formulation:

| Raw materials:                            | Pounds |
|-------------------------------------------|--------|
| Hydrogenated castor oil acids             | 7.58   |
| Arctic red oil                            | 7.58   |
| Hydrated lime                             | 2.12   |
| Water                                     | 0.32   |
| Caustic soda                              | 0.10   |
| Solvent extract from bright stock         | 66.13  |
| Solvent refined 200 viscosity neutral oil | 331.17 |

The grease was prepared according to the process of our invention as follows:

The procedure of Example I was followed except that the initial soap concentration in the base oil mixture was only 20% by weight. After preparation according to Example I, the remainder of the mineral oil was added to reduce the soap concentration to 4% by weight. At this point, the grease contained 0.134 weight percent of free fatty acid, calculated as oleic acid, and had an ASTM taper-hole disc worked penetration of 144. The grease was then further reduced by further addition of bright stock and neutral oil to soap concentrations of the following weight percentages: 1.12, 1.0, 0.80 and 0.62. At all tested concentrations of soap in the base oil, the greases exhibited exceptional stability and were excellent semi-fluid saddle lubricants for textile mill use. No difficulties were encountered in the preparation of said greases. Total time for the preparation of the greases was 16 hours.

#### Example III

A further non-limiting example of the grease of our invention and the process of preparation is a grease of the following formulation:

| Raw materials:                                                       | Grams  |
|----------------------------------------------------------------------|--------|
| Hydrogenated castor oil acids                                        | 114.8  |
| Arctic red oil                                                       | 114.8  |
| Hydrated lime                                                        | 30.6   |
| Water                                                                | 4.5    |
| Caustic soda                                                         | 1.5    |
| Acid-refined gulf coastal mineral oil (viscosity 120 SUS at 210° F.) | 5274.0 |

The procedure of Example I was followed, except for the substitution of the acid-treated gulf coastal mineral oil for the solvent refined bright stock and solvent refined neutral (200 viscosity) oil mixture. When the free fatty acid concentration was adjusted so that the grease at 20 weight percent concentration contained 0.3-1.85% by weight, calculated as oleic acid, free fatty acid, no processing difficulties were encountered, a high yield of satisfactory grease in a relatively short total process time, under six hours, was obtained, and the grease was compatible with all types of mineral oils.

The results of a series of comparative tests between greases of different formulations appear below in Example IV.

*Example IV*

| Raw Materials                                | Weight Percent |          |          |                        |
|----------------------------------------------|----------------|----------|----------|------------------------|
|                                              | Sample A       | Sample B | Sample C | Sample D               |
| 12-hydroxy stearic acid                      | 1.88           | 1.93     | 1.98     | 2.03                   |
| Arctic red oil                               | 1.88           | 1.93     | 1.98     | 2.03                   |
| Hydrated lime                                | 0.51           | 0.51     | 0.51     | 0.51                   |
| Water                                        | 0.075          | 0.075    | 0.075    | 0.075                  |
| Caustic soda                                 | 0.025          | 0.025    | 0.025    | 0.025                  |
| Intermediate viscosity index<br>bright stock | 83.20          | 83.12    | 83.03    | 82.93                  |
| 200 viscosity neutral oil                    | 12.43          | 12.41    | 12.40    | 12.39                  |
| Wt. Percent soaps                            | 4.0            | 4.0      | 4.0      | Could not be prepared. |
| Free fatty acids (as oleic acid):            |                |          |          |                        |
| Wt. percent at 32.7% soap concentration      | 2.25           | 2.30     | 3.03     | 3.37                   |
| Wt. percent at 20% soap concentration        | 1.38           | 1.41     | 1.85     | 2.06                   |
| Wt. percent at 4.0% soap concentration       | 0.42           | 0.43     | 0.52     | Could not be prepared. |
| Penetration, unworked <sup>1</sup>           | 186            | 151      | 162      | Could not be tested.   |
| Penetration, worked, 100 strokes             | 180            | 181      | 154      | Do.                    |

<sup>1</sup> Penetration performed by Tapered-Hole Disc method.

The procedure of the preceding examples was followed in the preparation of Samples A, B, C and D, except that the soaps were formed at 32.7% concentration in the base oil, rather than at 20% or 40%. The base oil consisted of about 64 weight percent bright stock and 36 weight percent neutral oil. After dehydration of the grease at 230-240° F., it in each case was cut back to 4.0 weight percent soap concentration with the balance of the mineral oils.

It is seen from a study of Example IV that a satisfactory grease can be obtained when the free fatty acid content during preparation of the grease is kept at a weight ratio to the soap concentration of about 1.38-1.85:20. When the free fatty acid-soap ratio went as high as 2.06:20 a satisfactory grease could not be prepared, the grease during processing separating into distinct layers and otherwise resisting blending. Satisfactory worked and unworked penetration values were obtained only for the greases prepared with free fatty acid contents not higher than 1.85 wt. percent, based on 20 wt. percent concentration of calcium soaps. The upper limit of the critical range of free fatty acids essential to satisfactory grease preparation has therefore been demonstrated. As previously shown, this range has a lower limit of approximately 0.3 wt. percent of free fatty acid per 20 wt. percent concentration of calcium soaps present.

The grease of our invention can be prepared with uniformity provided the free fatty acid content is controlled as above-described, that is, is kept during processing at a weight ratio to the gelation agent of 0.3-1.85:20. The grease of our invention can be cut back to as low as 0.50 weight percent concentration of soap while still retaining its lubricating properties, homogeneity, clarity and smoothness. At this concentration the grease is a semi-fluid product.

The soap of the grease of our invention, although pointed out in the above examples to be the calcium soaps of a mixture of hydrogenated castor oil acids or 12-hy-

droxy stearic acid and arctic red oil acids, is not limited to such. The required acids for reaction with the hydrated lime constitute 25-75% by weight of acids from the group consisting of saturated mono- and di-hydroxy fatty acids containing from eighteen to twenty four carbon atoms per molecule, and the remainder or 75-25% by weight consisting of acids from the group consisting of non-hydroxy fatty acids of the non-drying type having not more than one unsaturated linkage in the molecule and containing from eighteen to twenty four carbon atoms per molecule. As to the saturated acids, it is preferred to use those containing at least twenty carbon atoms per molecule because of the greater solubility of the calcium soaps of these acids in mineral oil. All of the soap present in the grease of our invention and utilized as the gelation agent consists of the calcium soaps of the above-defined two types of acids.

We claim and particularly point out as our invention:

1. An anhydrous calcium soap grease comprising viscous mineral oil treated with sufficient sodium hydroxide to neutralize naturally occurring acids and a gelation agent, substantially all of said gelation agent in the grease, except the soap resulting from the neutralization of the naturally occurring acids present in the mineral oil, consisting of calcium soaps of mixed acids from group (1) saturated mono-hydroxy fatty acids containing from eighteen to twenty four carbon atoms per molecule, and group (2) non-hydroxy fatty acids having not more than one unsaturated linkage in the molecule and containing from eighteen to twenty four carbon atoms per molecule, the group (1) acids constituting approximately 25-75 percent by weight of the mixed acids of said calcium soaps and the group (2) acids constituting approximately 75-25 percent by weight of the mixed acids of said calcium soaps and the gelation agent being present in an amount which will produce a gelled grease structure, and free fatty acids selected from the group consisting of above-defined group (1) acids and above-defined group (2) acids and mixtures thereof in a weight ratio to said gelation agent of 0.3-1.85:20.

2. A grease in accordance with claim 1 in which said gelation agent is present in the grease in an amount of at least 0.5 percent by weight and in which the free fatty acids amount to at least about 0.02 percent by weight.

3. A grease in accordance with claim 1 in which the group (2) acid has one double-bonded carbon to carbon linkage.

4. A grease in accordance with claim 1 in which the group (2) acid is saturated acid having at least twenty carbon atoms in the molecule.

5. A grease in accordance with claim 3 in which the group (1) acid is 12-hydroxy stearic acid.

6. A grease in accordance with claim 4 in which the group (1) acid is 12-hydroxy stearic acid.

7. A grease in accordance with claim 5 in which the group (2) acid is oleic acid.

8. A grease in accordance with claim 7 in which group (1) and group (2) acids of said gelation agent are present in approximately equal amounts.

9. The method of preparing anhydrous calcium soap grease which comprises the steps of mixing together a mineral lubricating oil fraction treated with sufficient sodium hydroxide to neutralize naturally occurring acids and at least one hydroxy fatty acid from group (1) acids consisting of saturated mono-hydroxy fatty acids having eighteen to twenty four carbon atoms per molecule and at least one non-hydroxy fatty acid from group (2) acids consisting of acids containing not more than one unsaturated linkage and having between eighteen and twenty four carbon atoms per molecule, said acids being present in an amount sufficient to gel said mineral lubricating oil fraction on conversion of said acids to calcium soaps, and being present in a ratio of 1-3 parts of group (1) acids to 3-1 parts by weight of group

(2) acids, adding to the mixture with concomitant heating to about 210-212° F. until foaming subsides sufficient lime to saponify said acids and providing free fatty acids in the mixture in a weight ratio to calcium soaps in said mixture of 0.3-1.85:20, and cooking the resulting mixture at 230°-275° F. until the grease is substantially completely dehydrated.

10. The method of claim 9 in which said lime substantially completely saponifies all said group (1) and group (2) acids in the mixture and in which said free fatty acids selected from the group consisting of group (1) and group (2) acids are thereafter added back to the soap-containing mixture in the desired amount.

11. The method of claim 9 in which said lime saponifies only a portion of said group (1) and group (2) acids present, the remaining portion of said group (1) and group (2) acids in desired amount being present as said free fatty acids.

12. The method in accordance with claim 9 in which group (1) acid and group (2) acid before reaction with said lime are present in the mixture in approximately equal amounts, in which the resulting calcium soaps are present during said grease preparation in approximately twenty percent by weight, in which said free fatty acids consist essentially of approximately equal amounts of acid from group (1) acids and acid from group (2) acids and the total free fatty acid concentration during said

5 grease preparation is about 0.8 percent by weight and in which said grease base is blended with mineral lubricating oil to a final calcium soap content of about 4 percent by weight and a final free fatty acid content of about 0.16 percent by weight.

13. The method in accordance with claim 10 in which said group (1) acid of said soap and said free fatty acid is 12-hydroxy stearic acid and in which said group (2) acid of said soap and said free fatty acid is oleic acid.

#### References Cited in the file of this patent

#### UNITED STATES PATENTS

|           |                      |                |
|-----------|----------------------|----------------|
| 2,358,939 | Nelson et al. _____  | Sept. 26, 1944 |
| 2,413,121 | Swenson _____        | Dec. 24, 1946  |
| 2,413,122 | Swenson _____        | Dec. 24, 1946  |
| 2,450,220 | Ashburn et al. _____ | Sept. 28, 1948 |
| 2,475,589 | Bondi _____          | July 12, 1949  |
| 2,607,735 | Sproule et al. _____ | Aug. 19, 1952  |
| 2,613,182 | Sproule et al. _____ | Oct. 7, 1952   |

#### OTHER REFERENCES

Manufacture and Application of Lubricating Greases,  
25 Boner, Reinhold Pub. Corp., N.Y. (1954), pp. 46, 47,  
388 and 392.